# EUROPEAN PATENT SPECIFICATION

(11) **EP 1 803 797 B1**
(45) Date of publication and mention of the grant of the patent: **03.12.2014**
(21) Application number: 06256586.6
(22) Date of filing: 27.12.2006
(51) Int. Cl.: C10M 163/00, C10M 159/16, C10N 40/25

(54) **Use of a lubricating oil composition for improving the acrylic rubber sealant compatability in an internal combustion engine**
Verwendung einer Schmiermittelzusammensetzung zur Erhöhung der Acrylkautschukdichtungskompatibilität bei einem Verbrennungsmotor
Utilisation d'une composition lubrifiante pour améliorer la compatibilité d'un matériau d'étanchéité en caoutchouc acrylique dans un moteur à combustion interne

(30) Priority: 27.12.2005 JP 2005375974
(43) Date of publication of application: 04.07.2007
(73) Proprietor: Chevron Japan Ltd., Chiyoda-ku, Tokyo 101-0041 (JP)
(72) Inventor: Takeuchi, Yoshitaka, Haibara-gun, Shizuoka (JP); Yamashita, Yoshito, Omaezaki-shi, Shizuoka (JP); Nakazato, Morikuni, Omaezaki-shi, Shizuoka (JP)
(74) Representative: Nash, David Allan

(56) References cited:
- EP-A2- 1 167 497
- EP-A2- 1 452 581
- US-A1- 2004 102 335

## Description

The present invention relates to use of a lubricating oil composition for improving the acrylic rubber sealant compatibility with the lubricating oil composition in operation of an internal combustion engine.

### BACKGROUND OF THE INVENTION

In mechanical devices such as internal-combustion engine vehicles and various other industrial machines, it is necessary to supply a lubricating oil to mechanisms involving rubbing movement. Lubrication systems for supplying a lubricating oil are generally equipped with various sealing materials (sealants). Examples of the sealing materials include resin or rubber sealants such as silicone rubber sealant, acrylic rubber sealant, fluorocarbon resin sealant, nitrile rubber sealant, hydrogenated nitrile rubber sealant and ethylene-propylene rubber sealant. According to their physical and chemical characteristics, those sealants are optionally selected to be installed in proper parts of the lubrication systems. Among the above-mentioned materials, acrylic rubber sealant is particularly used as packing parts for fixation because it is not only excellent in heat resistance and oil resistance but also inexpensive,

At the present time, it is required to improve lubricating oils for the purpose of meeting certain performance requirements. Most lubricating oils contacting rubbing mechanisms in various machines are nowadays high-performance lubricating oil compositions comprising a lubricating base oil and various additives added thereto.

However, lubricating oil compositions containing various additives often deteriorate resin or rubber sealants despite satisfying lubricating performance requirements. Most of the additives contained in the compositions are so chemically active that they are liable to shrink the sealants and/or to impair their strength and elasticity.

Accordingly, it is desirable to have a lubricating oil composition which satisfies the severe performance requirements concerning lubricating oil compositions and, at the same time, which hardly impairs sealing performance of the sealants themselves.

U.S. Patent No. 6,124,247 describes a lubricating oil composition containing a borated glycerol ester and a mono-succinimide or bis-succinimide type dispersant subjected or not subjected to post-treatment with, for example, ethylene carbonate. It is stated that this oil composition has excellent compatibility with fluorocarbon elastomer, which is used as a sealant in a lubrication system of an internal-combustion engine.

JP-A-11-181461 describes that a lubricating oil composition containing an aliphatic amine has excellent compatibility with rubber sealants.

U.S. Patent No. 6,569,818 describes a lubricating oil composition containing an ashless dispersant of an alkenyl- or alkyl-succinic imide or a derivative thereof, an alkali metal or alkaline earth metal alkylsalicylate of non-sulfide or otherwise an alkali metal salt of alkylphenol derivative having a Mannich base structure, a zinc dialkyldithiophosphate, and an oxidation inhibiting phenol or amine compound. It is stated that all of the ash content, the phosphorus content and the sulfur content of the disclosed lubricating oil composition are low levels and that the lubricating oil composition gives high detergency at a high temperature. U.S. Patent No. 6,569,818, however, is silent about a lubricating oil composition of the present invention described hereinbelow. Further, this reference neither describes nor suggests any effect that the lubricating oil composition has on sealants.

EP 1 452 581 A2 provides a method of improving elastomer seal compatibility and dispersancy in an internal combustion engine, said method comprising contacting the elastomer seal in the internal combustion engine with a lubricating oil composition comprising: a) a major amount of a base oil of lubricating viscosity; b) a carboxylated detergent-dispersant obtained by: (i) neutralizing alkylphenols using an alkaline earth base in the presence of at least one carboxylic acid that contains from one to four carbon atoms but in the absence of alkali base, dialcohol, and monoalcohol, forming an intermediate product; and (ii) carboxylating the intermediate product using carbon dioxide so that at least 20 mole percent of the original alkylphenol starting material has been converted to alkaline earth metal single aromatic-ring hydrocarbyl salicylate; and c) a nitrogen-containing dispersant. The nitrogen-containing dispersant employed in the lubricating oil composition of EP 1 452 581 A2 is an ashless dispersant such as an alkenyl succinimide, an alkenyl succinic anhydride, an alkenyl succinate ester, and the like, or mixtures of such dispersants.

### SUMMARY OF THE INVENTION

The present invention relates to use of a lubricating oil composition for improving acrylic rubber sealant compatibility with the lubricating oil composition in operation of an internal combustion engine, wherein the lubricating oil composition comprises:
a) a major amount of a base oil of lubricating viscosity,
b) a nitrogen-containing ashless dispersant in an amount of 0.01 to 0.3 wt.%, preferably 0.01 to 0.1 wt.%, in terms of the nitrogen content, based on the total amount of the lubricating oil composition,
c) a metal-containing detergent of an alkali metal or alkaline earth metal salt of alkylphenol derivative having a Mannich base structure in an amount of 0.001 to 0.4 wt.%, preferably 0.002 to 0.1 wt.%, in terms of the metal content, based on the total amount of the lubricating oil composition, and
d) a phosphorus-containing organic compound in an amount of 0.001 to 0.5 wt.%, preferably 0.01 to 0.2 wt.%, in terms of the phosphorus content, based on the total amount of the lubricating oil composition,
wherein the ratio of components b) to c) is in the range of from 1:0.005 to 1:2, preferably 0:0.01 to 1:0.3, in terms of the nitrogen content;
and wherein the improvement in acrylic rubber sealant compatibility is an improvement in elongation change as measured using the CEC-L-39-T-96 affinity test for sealing rubber.

The nitrogen-containing ashless dispersant in the lubricating oil composition employed in the present invention is an alkenyl- or alkyl-succinic imide or a derivative thereof.

The metal-containing detergent of an alkali metal or alkaline earth metal salt of alkylphenol derivative in the lubricating oil composition employed in the present invention has a Mannich base structure represented by the following formula: wherein R is an alkyl group having 8 to 30 carbon atoms, and n is 0 or a positive integer.

The lubricating oil composition employed in the present invention may further comprise a phosphorus-containing organic compound selected from the group consisting of zinc dihydrocarbyldithiophosphates, zinc dihydrocarbylphosphates, phosphoric acid esters, phosphorous acid esters, and thiophosphoric acid esters.

The lubricating oil composition employed in the present invention may further comprise a metal-containing detergent selected from the group consisting of alkali metal or alkaline earth metal salicylates, carboxylates, phenates and sulfonates in an amount of 1.0 wt.% or less in terms of the metal content.

The amount of metal-containing detergent selected from the group consisting of alkali metal or alkaline earth metal salicylates, carboxylates, phenates and sulfonates to the amount of metal-containing detergent of an alkali metal or alkaline earth metal salt of alkylphenol derivative having a Mannich base structure is in a ratio of 1:0.003 to 1:1 in terms of the metal content.

The lubricating oil composition employed in the present invention may further comprise a molybdenum compound selected from the group consisting of an oxymolybdenum complex prepared by the reaction between an acidic molybdenum compound and a basic nitrogen compound, sulfurized oxymolybdenum dithiocarbamate, and sulfurized oxymolybdenum dithiophosphate, in amount of 0.25 wt.% or less in terms of the molybdenum content.

The lubricating oil composition employed in the present invention may further comprise an alkali metal borate in an amount of 2 wt.% or less and an oxidation inhibitor selected from the group consisting of hindered phenol compounds and diarylamine compounds in an amount of 5 wt.% or less.

The base oil of lubricating viscosity contains 10 wt.% or more of a mineral oil showing the following characteristics:
- 17 wt.% or less evaporation loss according to ASTM D-5800,
- 90 wt.% or more saturated content,
- 10 wt.% or less, aromatic component,
- 0.01 wt.% or less, sulfur content, and
- 120 or more viscosity index.

The lubricating oil composition employed in the present invention is a SAE viscosity grade selected from the group consisting of 0W20, 0W30, 5W20, 5W30 and 10W30. Preferably, the lubricating oil composition meets the SAE 10W-30 viscosity grade.

Further, it has been discovered that a lubricating oil composition containing a certain combination of a nitrogen-containing dispersant and a metal-containing detergent of an alkali metal salt of alkylphenol derivative having a Mannich base structure, together with a phosphorus-containing organic compound, can be effectively employed for improving the acrylic rubber sealant compatibility in an internal combustion engine, if the ratio of the nitrogen-containing dispersant and a metal-containing detergent of an alkali metal salt of alkylphenol derivative having a Mannich base structure is adjusted to a specific range, i.e., in the range of from 1:0.005 to 1:2 in terms of the nitrogen content. The lubricating oil composition hardly impairs the sealing performance of the acrylic rubber sealant.

### DETAILED DESCRIPTION OF THE INVENTION

The present invention resides in use of a certain lubricating oil composition to improve the acrylic rubber sealant compatibility with the lubricating oil composition in operation of an internal combustion engine. The lubricating oil composition, while meeting the lubricating performance requirements of internal combustion engines, at the same time is less detrimental to the sealing performance of acrylic rubber sealants found in internal combustion engines as compared to conventionally used lubricating oil compositions. Thus, the present invention advantageously improves the acrylic rubber sealant compatibility in internal combustion engines.

The preferred embodiments of the present invention will be described in further detail below. It should be noted that when weight percent is used herein, it is based on the total weight percent of the lubricating oil composition unless otherwise specified.

The lubricating oil composition employed in the present invention will contain a nitrogen-containing ashless dispersant. The nitrogen-containing ashless dispersant is preferably is a polyolefin-derived alkenyl- or alkyl-succinic imide or a derivative thereof. The amount of the nitrogen-containing ashless dispersant is in the range of 0.01 to 0.3 wt.%, preferably 0.01 to 0.1wt.%, in terms of the nitrogen content, based on the total amount of the lubricating oil composition.

A representative succinic imide can be prepared by the reaction between succinic anhydride having a high molecular weight alkenyl or alkyl substituent group with polyalkylenepolyamine containing 4 to 10 nitrogen atoms on average, preferably 5 to 7 nitrogen atoms. The high molecular weight alkenyl or alkyl substituent group is preferably a polybutene having a number average molecular weight of approximately 900 to 5,000.

The process for preparing the polybutenylsuccinic anhydride by the reaction between polybutene and maleic anhydride is generally performed by a chlorination method utilizing chlorine. While this reaction is advantageous in giving a high reaction yield, it has a disadvantageous feature in that a large amount (for instance, approximately 2,000 to 3,000 ppm) of chlorine remains in the final succinic imide product. In contrast, a thermal reaction process utilizing no chlorine can give a final reaction product having an extremely low chlorine content (such as 0 to 30 ppm). It is, therefore, preferred to use a succinic imide derived from the polybutenylsuccinic anhydride prepared by the thermal reaction process so that the chlorine content can be in the range of 0 to 30 ppm. The resulting succinic imide can be further converted into a modified succinic imide by a further reaction with boric acid, alcohol, aldehyde, ketone, alkylphenol, cyclic carbonate or organic acids. From the thermal stability and oxidation stability, particularly preferred is a boron-containing alkenyl- or alkyl-succinic imide which is produced by the reaction with boric acid or a boron-containing compound.

The lubricating oil composition employed in the present invention indispensably contains the ashless dispersant, whose representative example is an alkenyl- or alkyl-succinic imide or a derivative thereof. As the ashless dispersant, ashless dispersants of alkenylbenzylamine type and alkenylsuccinic acid ester type can be also used.

The lubricating oil composition employed in the present invention will contain metal-containing detergent of an alkali metal or alkaline metal earth metal salt of alkylphenol derivative. The metal-containing detergent of an alkali metal or alkaline metal earth metal salt of alkylphenol derivative has a Mannich base structure represented by the following formula:

The amount of the metal-containing detergent of an alkali metal or alkaline earth metal salt of alkylphenol derivative having a Mannich base structure is in the range of 0.001 to 0.4 wt.% in terms of the metal content or 0.002 to 0.1 wt.% in terms of the nitrogen content, based on the total amount of the lubricating oil composition.

The metal-containing detergent of an alkali metal (e.g., sodium, potassium) or alkaline earth metal (e.g., calcium, barium, magnesium) salt of alkylphenol derivative having a Mannich base structure, is generally prepared by the steps of:
synthesizing an intermediate having aminomethylated phenol ring by Mannich reaction from alkylphenol, formaldehyde, amine or an amine compound; and
neutralizing the synthesized intermediate with a base such as calcium hydroxide to covert it into a metal salt. Examples include the compound of the above formula having the following characteristics:
   Ca content: 2.5 wt.%,
   N content: 1.6 wt.%,
   total base number: 135 mg•KOH/g, and
   base number attributable to basic nitrogen: approximately 50% of the total base number.

The ratio of the nitrogen-containing ashless dispersant to the metal-containing detergent of an alkali metal or alkaline earth metal salt of alkylphenol derivative having a Mannich base structure is in the range of from 1:0.005 to 1:2, preferably 1:0.01 to 1:0.3, in terms of the nitrogen content.

The lubricating oil composition employed in the present invention will contain a phosphorus-containing organic compound selected from the group consisting of zinc dihydrocarbyldithiophosphates, zinc dihydrocarbylphosphates, phosphoric acid esters, phosphorous acid esters, and thiophosphoric acid esters. The amount of the phosphorus-containing organic compound is in the range of 0.001 to 0.5 wt.%, preferably 0.01 to 0.2 wt.%, in terms of the phosphorus content, based on the total amount of the lubricating oil composition.

Examples of the phosphorus-containing organic compounds include zinc dihydrocarbyldithiophosphates, zinc dihydrocarbylphosphates, phosphoric acid esters, phosphorous acid esters, and thiophosphoric acid esters in which each ester is generally derived from the corresponding acid and an alkylalcohol having 3 to 18 carbon atoms or an alkylarylalcohol having an alkyl group of 3 to 18 carbon atoms. If a zinc dihydrocarbyldithiophosphate (zinc dialkyldithiophosphate) is added, the amount of the additive is preferably in the range of 0.01 to 0.1 wt.% in terms of the phosphorus content, based on the total amount of the lubricating oil composition. From the viewpoint of reducing the phosphorus content and the sulfur content, the amount preferably is in the range of 0.01 to 0.06 wt.%, based on the total amount of the lubricating oil composition.

The zinc dialkyldithiophosphate preferably has an alkyl group of 3 to 18 carbon atoms or an alkylaryl group having an alkyl group of 3 to 18 carbon atoms. It is particularly preferred for the zinc dialkyldithiophosphate to have an alkyl group derived from a secondary alcohol having 3 to 18 carbon atoms or an alkyl group derived from a mixture of a primary alcohol having 3 to 18 carbon atoms and a secondary alcohol having 3 to 18 carbon atoms, because the zinc dialkyldithiophosphate having that alkyl group is particularly effective in wear reduction. A zinc dialkyldithiophosphate derived from a primary alcohol is also excellent in heat resistance. The zinc dithiophosphates can be used singly, but it is preferred to use a mixture mainly comprising a secondary alkyl-type and/or a primary alkyl type.

The lubricating oil composition employed in the present invention may further contain another metal-containing detergent selected from the group consisting of alkali metal or alkaline earth metal salicylates, carboxylates, phenates and sulfonates in an amount of 1.0 wt.% or less in terms of the metal content, based on the total amount of the lubricating oil composition.

The amount of the metal-containing detergent selected from the group consisting of alkali metal or alkaline earth metal salicylates, carboxylates, phenates and sulfonates to the amount of the metal-containing detergent of an alkali metal or alkaline earth metal salt of alkylphenol derivative having a Mannich base structure is in a ratio of 1:0.003 to 1:1 in terms of the metal content, based on the total amount of the lubricating oil composition.

The lubricating oil composition employed in the present invention may further contain an oxidation inhibitor selected from the group consisting of hindered phenol compounds and diarylamine compounds in an amount of 5 wt.% or less, based on the total amount of the lubricating oil composition. In view of having a base number attributable to nitrogen, diarylamine-type oxidation inhibitors are particularly advantageous. On the other hand, however, hindered phenol-type oxidation inhibitors effectively prevent deterioration caused by NOₓ oxidation.

Examples of the hindered phenol oxidation inhibitors include 2,6-di-t-butyl-p-cresol, 4,4'-methylenebis(2,6-di-t-butylphenol), 4,4'-methylenebis(6-t-butyl-o-cresol), 4,4'-isopropylidenebis(2,6-di-t-butylphenol), 4,4'-bis(2,6-di-t-butylphenol), 2,2'-methylenebis(4-methyl-6-t-butylphenol), 4,4'-thiobis(2-methyl-6-t-butylphenol), 2,2-thiodiethylenebis[3-(3,5-di-t-butyl-4-hydroxyphenyl)propionate], octyl 3-(3,5-di-t-butyl-4-hydroxyphenyl)propionate, and octadecyl 3-(3,5-di-t-butyl-4-hydroxyphenyl)propionate.

Examples of the diarylamine oxidation inhibitors include an alkyldiphenylamine containing a mixture of alkyl groups having 4 to 9 carbon atoms, p,p'-dioctyldiphenylamine, phenyl-α-naphthylamine, phenyl-α-naphthylamine, alkylated α-naphthylamine, and alkylated phenyl-α-naphthylamine.

Each of the hindered phenol compounds and the diarylamine compounds can be used singly or in combination. Other oil soluble oxidation inhibitors can be employed in combination.

The lubricating oil composition employed in the present invention may further contain a molybdenum compound selected from the group consisting of an oxymolybdenum complex prepared by the reaction between an acidic molybdenum compound and a basic nitrogen compound, sulfurized oxymolybdenum dithiocarbamate, and sulfurized oxymolybdenum dithiophosphate, in an amount of 0.25 wt.% or less in terms of the molybdenum content, based on the total amount of the lubricating oil composition.

The molybdenum-containing compound mainly functions as a friction modifier, an oxidation inhibitor or an anti-wear agent in the lubricating oil composition employed in the present invention. In addition, it also improves detergency at a high temperature. The molybdenum-containing compound is preferably in an amount of 10 to 2,500 ppm in terms of the molybdenum content. Examples of the molybdenum-containing compounds include sulfur-containing molybdenum complex of succinimide, sulfurized oxymolybdenum dithiocarbamate, sulfurized oxymolybdenum dithiophosphate, amine molybdenum complex compound, oxymolybdenum diethylate amide, and oxymolybdenum monoglyceride. Sulfur-containing molybdenum complex of succinimide is particularly effective in improving the detergency at a high temperature.

The lubricating oil composition employed in the present invention may further contain an alkali metal borate in an amount of 2 wt.% or less, based on the total amount of the lubricating oil composition. The alkali metal borate hydrate is also effective in improving the detergency at a high temperature and in giving a base number. The term "alkali metal borate hydrate" in the present invention means a compound representatively prepared by the method disclosed in U.S. Patent Nos. 3,929,650 and 4,089,790. For example, it can be obtained by the steps of carbonating a neutral alkali metal or alkaline earth metal sulfonate in the presence of an alkali metal hydroxide to prepare a basic sulfonate; and making the basic sulfonate to react with boric acid, to prepare an alkali metal borate in the form of dispersed fine particles. The carbonation reaction is preferably conducted further in the presence of an ashless dispersant such as succinic imide. The alkali metal preferably is potassium or sodium. An example of the alkali metal borate hydrate additive is a suspension comprising a mixture of neutral calcium sulfonate and succinic imide and fine particles of KB₃O₅•H₂O having sizes of approximately 0.3 µm or less. The potassium can be replaced with sodium. The additive is also preferably used in consideration of water resistance.

The lubricating oil composition employed in the present invention may further contain a viscosity index improver in an amount of 20 wt.% or less, preferably 1 to 20 wt.%, based on the total amount of the lubricating oil composition. Examples of the viscosity index improver include polymer compounds such as polyalkyl methacrylate, ethylene-propylene copolymer, styrene-butadiene copolymer, and polyisoprene. Also employable are dispersant-type viscosity index improvers, which can be obtained by modifying the above polymers so that they can function as dispersants, and multi-functional viscosity index improvers. The viscosity index improvers can be used singly or in combination.

The lubricating oil composition employed in the present invention may further contain various other auxiliary additives. Examples of the auxiliary additives include zinc dithiocarbamate, methylenebis(dibutyldithiocarbamate), an oil-soluble copper compound, a sulfur-containing compound (e.g., sulfurized olefin, sulfurized ester, polysulfide), and an organic amide compound (e.g., oleyl amide). They function as oxidation inhibitors or anti-wear agents. It is also preferred to incorporate metal deactivators such as benzotriazole compounds and thiadiazole compounds. Further, a nonionic surface active agent of polyoxyalkylene such as a copolymer of polyoxyethylenealkylphenyl ether, ethylene oxide and propylene oxide can be added as a rust preventing agent or an demulsifier. It is also possible to incorporate various amines, amides, amine salts or derivatives thereof, and aliphatic acid esters of polyhydric alcohols or their derivatives. They serve as friction modifiers. It is further possible to incorporate various compounds that function as defoaming agents or pour point depressants. Each auxiliary additive is added to the lubricating oil composition employed in the present invention preferably in an amount of 3 wt.% or less, preferably 0.001 to 3 wt.% , based on the total amount of the lubricating oil composition.

### Base Oil of Lubricating Viscosity

The base oil used in the lubricating oil composition employed in the present invention generally is a mineral or synthetic oil showing a kinematic viscosity of 2 to 50 mm²/s at 100°C. There are no specific conditions with respect to the mineral or synthetic oil, but the base oil has a sulfur content of preferably 0.1 wt.% or less, more preferably 0.03 wt.% or less, most preferably 0.005 wt.% or less.

The mineral base oil is preferably subjected to properly combined treatments. For example, the mineral lubricant distillate thereof is preferably subjected to treatments such as solvent refining and hydrogenation processing in combination. In the present invention, it is preferred to use a highly hydrogen-refined (hydrocracked) base oil (having, for example, a viscosity index of 100 to 150, an aromatic component content of 5 wt.% or less, a nitrogen content of 50 ppm or less, and a sulfur content of 50 ppm or less). Examples include a high viscosity index-base oil prepared by isomerization or hydrocracking of synthetic wax synthesized from slack wax (crude wax) of mineral oil or natural gas.

It is particularly preferred that the base oil of lubricating viscosity is a mineral oil showing the following characteristics:
evaporation loss (ASTM D-5800): 17 wt.% or less,
content of saturated component: 90 wt.% or more,
content of aromatic component: 10 wt.% or less,
sulfur content: 0.01 wt.% or less, and
viscosity index: 120 or more;
or otherwise that the base oil of lubricating viscosity is a mineral oil mixture containing 10 wt.% or more of the above-mentioned mineral oil.
Examples of the synthetic oils (synthetic lubricant base oil) include a poly-α-olefin (copolymer of α-olefin having 3 to 12 carbon atoms), a dialkyl diester (ester derived from an alcohol having 4 to 18 carbon atoms and a dibasic acid such as adipic acid, azelaic acid or sebacic acid) such as dioctyl sebacate, a polyol ester (ester derived from a monobasic acid having 3 to 18 carbon atoms and 1-trimethylolpropane or pentaerythritol), and an alkylbenzene having an alkyl group of 9 to 40 carbon atoms.

Any of the above mineral or synthetic base oils may be used singly, but two or more of the mineral base oils or two or more of the synthetic base oils can be used in combination, if desired. Further, the mineral and synthetic base oils can be used in combination at any ratios, if desired, to prepare the appropriate base oil of lubricating viscosity.

It is preferred to use a major amount of base oil of lubricating viscosity in the lubricating oil composition employed in the present invention. A major amount of base oil of lubricating viscosity as defined herein comprises 40 wt % or more. Preferred amounts of base oil comprise 40 to 99.9 wt %, preferably greater than 50 to 97 wt %, more preferably 60 to 97 wt % of the lubricating oil composition.

The lubricating oil composition employed in the present invention can be prepared by adding the additives independently or all at once to the base oil. Otherwise, an additive concentrate comprising the additives in high concentrations can be beforehand prepared and then mixed it with a base oil to prepare the lubricating oil composition employed in the present invention.

### EXAMPLES

The base oil of lubricating viscosity and the additives used in the below-described Examples and Comparative Example are as follows:
(1) Base oil of lubricating viscosity
   Solvent refined base oil (A) (kinematic viscosity: 4.9 mm²/s at 100°C, viscosity index: 103, evaporation loss (ASTM D5800): 13 wt.%, sulfur content: 0.19 wt.%, content of saturated component: 70 wt.%) and solvent refined base oil (B) (kinematic viscosity: 10.8 mm²/s at 100°C, viscosity index: 97, evaporation loss (ASTM D5800): 2.3 wt.%, sulfur content: 0.22 wt.%, content of saturated component: 68 wt.%) were mixed in the ratio of 88:12 by weight to use.
(2) Additives
   Dispersant A: ethylene carbonate-treated succinimide dispersant [N content: 1.0 wt.%, CI content: 30 ppm by weight] which was prepared by the steps of:
      a) reacting a polybutene having a number average molecular weight of approximately 2,300 and 50% or more of methylvinylidene structure with maleic anhydride according to the thermal process, to produce an intermediate product;
      b) reacting the intermediate product with a polyalkylenepolyamine containing 6.5 nitrogen atoms (in one molecule) on average, to prepare succinimide of bis-form; and then
      c) treating the succinimide of bis-form with ethylene carbonate.
   Dispersant B: boron-containing succinimide dispersant [N content: 1.95 wt.%, B content: 0.66 wt.%, Cl content: less than 5 ppm by weight] which was prepared by the steps of:
      a) reacting a polybutene having a number average molecular weight of approximately 1,300 and 50% or more of methylvinylidene structure) with maleic anhydride according to the thermal process, to produce an intermediate product;
      b) reacting the intermediate product with a polyalkylenepolyamine containing 6.5 nitrogen atoms (in one molecule) on average, to prepare succinimide of bis-form; and then
      c) treating the succinimide of bis-form with boric acid.
   Detergent A: Mannich base calcium phenate (Ca: 2.5 wt.%, N: 1.6 wt.%, S: 0.1 wt.%, TBN: 135 mg•KOH/g).
   Detergent B: overbased sulfurized calcium phenate (Ca: 9.25 wt.%, S: 3.4 wt.%, TBN: 255 mg•KOH/g).
   Detergent C: overbased calcium sulfonate (Ca: 16.1 wt.%, TBN: 425 mg•KOH/g).
   Detergent D: basic calcium sulfonate (Ca: 2.35 wt.%, TBN: 17 mg•KOH/g).
   ZnDTP-1: zinc dialkyldithiophosphate (P: 7.2 wt.%, Zn: 7.85 wt.%, S: 14.4 wt.%, starting material: a secondary alcohol having 3 to 6 carbon atoms).
   ZnDTP-2: zinc dialkyldithiophosphate (P: 7.3 wt.%, Zn: 8.4 wt.%, S: 14 wt.%, starting material: a primary alcohol having 8 carbon atoms).
   Oxidation inhibitor: dialkyldiphenylamine (alkyl group: mixture of C₄-alkyl and C₈-alkyl groups, N: 4.6 wt.%, TBN: 180 mg•KOH/g).
   Mo compound: sulfur-containing molybdenum-succinimide complex (Mo: 5.5 wt.%, S: 0.2 wt.%, N: 1.6 wt.%, TBN: 10 mg•KOH/g).
      Alkali metal borate: dispersed fine particles of potassium borate hydrate (K: 8.3 wt.%, B: 6.8 wt.%, S: 0.26 wt.%, TBN: 125 mg•KOH/g).
   Viscosity index improver (VII): ethylenepropylene copolymer of non-dispersant type.
   Pour point depressant (PPD): polymethacrylic compound.

### Example 1

The below-mentioned additives and the base oil of lubricating viscosity were mixed to give the lubricating oil composition employed in the present invention. The lubricating oil composition was SAE viscosity grade 10W30. Also shown below are the contents of each element (Ca, P, N) in the lubricating oil composition, the ratio between the nitrogen content attributable to all the dispersants and that attributable to the detergent A (Mannich base calcium phenate), and the ratio between the metal content attributable to all the detergents and that attributable to the detergent A (Mannich base calcium phenate).
(1) Additives
   Dispersant A (amount: 3.0 wt.%, content in terms of nitrogen: 0.03 wt.%),
   Dispersant B (amount: 1.5 wt.%, content in terms of nitrogen: 0.03 wt.%),
   Detergent A (amount: 0.4 wt.%, content in terms of calcium: 0.01 wt.%, content in terms of nitrogen: 0.006 wt.%),
   Detergent B (amount: 0.86 wt.%, content in terms of calcium: 0.08 wt.%),
   Detergent C (amount: 0.87 wt.%, content in terms of calcium: 0.14 wt.%),
   Detergent D (amount: 0.43 wt.%, content in terms of calcium: 0.01 wt.%),
   ZnDTP-1 (amount: 0.97 wt.%, content in terms of phosphorus: 0.07 wt.%),
   ZnDTP-2 (amount: 0.41 wt.%, content in terms of phosphorus: 0.03 wt.%),
   Oxidation inhibitor (amount: 0.2 wt.%),
   Mo compound (amount: 0.15 wt.%, content in terms of molybdenum: 83 ppm by weight),
   Alkali metal borate (amount: 0.25 wt.%),
   Viscosity index improver (VII, amount: 6.3 wt.%), and
   Pour point depressant (PPD, amount: 0.3 wt.%).
(2) Base oil of lubricating viscosity (amount: residual amount)
(3) Content of each element (Ca, P, N) in the lubricating oil composition
   Calcium (Ca): 0.24 wt.%, Phosphorus (P): 0.10 wt.%, Nitrogen (N): 0.08 wt.%
(4) Ratio of the nitrogen content attributable to all the dispersants to that attributable to the detergent A (Mannich base calcium phenate): 1:0.1
(5) Ratio of the metal content attributable to all the detergents in the composition to that attributable to the detergent A (Mannich base calcium phenate): 1:0.04

### Example 2

The procedures of Example 1 were repeated except for changing the amount of the detergent A (Mannich base calcium phenate) into 1.16 wt.% (content in terms of calcium: 0.03 wt.%, content in terms of nitrogen: 0.018 wt.%) and for changing the residual amount of the base oil of lubricating viscosity so that the total amount of the lubricating oil composition is 100 wt.%. The prepared lubricating oil composition was SAE viscosity grade 10W30. Shown below are the contents of each element (Ca, P, N) in the lubricating oil composition, a ratio between the nitrogen content attributable to all the dispersants and that attributable to the detergent A (Mannich base calcium phenate), and a ratio between the metal content attributable to all the detergents and that attributable to the detergent A (Mannich base calcium phenate).
(1) Contents of each element (Ca, P, N) in the lubricating oil composition Calcium (Ca): 0.26 wt.%, Phosphorus (P): 0.10 wt.%, Nitrogen (N): 0.09 wt. %
(2) Ratio of the nitrogen content attributable to all the dispersants to that attributable to the detergent A (Mannich base calcium phenate): 1:0.3
(3) Ratio of the metal content attributable to all the detergents in the lubricating oil composition to that attributable to the detergent A (Mannich base calcium phenate): 1:0.12

### Comparative Example A

Comparative Example A was prepared according to the procedures of Example 1 except for not adding the detergent A (Mannich base calcium phenate) and for changing the amount of the base oil of lubricating viscosity so that the total amount of the lubricating oil composition is 100 wt.%. The prepared lubricating oil composition was SAE viscosity grade 10W30. The contents of each element (Ca, P, N) in the lubricating oil composition are shown below.
(1) Contents of each element (Ca, P, N) in the lubricating oil composition Calcium (Ca): 0.23 wt.%, Phosphorus (P): 0.10 wt.%, Nitrogen (N): 0.07 wt.%

### Evaluation of Compatibility With Acrylic Rubber Sealant

According to the affinity test for sealing rubber (CEC-L-39-T-96), compatibility with acrylic rubber was evaluated in the following manner. A piece of RE2-99 (acrylic rubber) was immersed in the lubricating oil composition to be tested at 150°C for 7 days, and then the degree of deterioration of the acrylic rubber piece was evaluated. The results are set forth in Table 1. In Table 1, the pass limits specified in JASO (Japanese Automobile Standard Organization) M355-2005 are also shown.

**Table 1.**

| | Pass Limit | Example 1 | Example 2 | Comparative Example A |
|---|---|---|---|---|
| Volume change(%) | -7 to +5 | +2 | 0 | +2 |
| Hardness change | -5 to +8 | +3 | +4 | +3 |
| Tensile strength change(%) | -15 to +18 | +2 | +2 | -4 |
| Elongation change(%) | -35 to +10 | -23 | -19 | -35 |

The above results shown in Table 1 indicate that both the lubricating oil compositions of the present invention (Examples 1 and 2) and that for Comparative Example A satisfy the JASO standards. It is also shown that the lubricating oil compositions of the present invention were remarkably improved in the elongation change, as compared with the lubricating oil composition for comparative example.

## Claims

1. Use of a lubricating oil composition for improving the acrylic rubber sealant compatibility with the lubricating oil composition in operation of an internal combustion engine, wherein the lubricating oil composition comprises:
a) a major amount of a base oil of lubricating viscosity,
b) a nitrogen-containing ashless dispersant in an amount of 0.01 to 0.3 wt. % in terms of the nitrogen content, based on the total amount of the lubricating oil composition,
c) a metal-containing detergent of an alkali metal or alkaline earth metal salt of alkylphenol derivative having a Mannich base structure in an amount of 0.001 to 0.04 wt. % in terms of the metal content, based on the total amount of the lubricating oil composition, and
d) a phosphorus-containing organic compound in an amount of 0.001 to 0.5 wt. % in terms of the phosphorus content, based on the total amount of the lubricating oil composition,
wherein the ratio of components b) to c) is in the range of from 1:0.005 to 1:2 in terms of the nitrogen content;
and wherein the improvement in acrylic rubber sealant compatability is an improvement in elongation change as measured using the CEC-L-39-T-96 affinity test for sealing rubber.

2. The use according to claim 1, wherein the nitrogen-containing ashless dispersant is an alkenyl- or alkyl-succinic imide or a derivative thereof.

3. The use according to claim 1, wherein the metal-containing detergent of an alkali metal or alkaline earth metal salt of alkylphenol derivative having a Mannich base structure is represented by the following formula: wherein R is an alkyl group having 8 to 30 carbon atoms, and n is 0 or a positive integer.

4. The use according to claim 1, wherein the phosphorus-containing organic compound is selected from the group consisting of zinc dihydrocarbyldithiophosphates, zinc dihydrocarbylphosphates, phosphoric acid esters, phosphorous acid esters, and thiophosphoric acid esters.

5. The use according to claim 1, wherein the amount of the nitrogen-containing ashless dispersant is in the range of 0.01 to 0.1 wt. % in terms of the nitrogen content, based on the total amount of the lubricating oil composition.

6. The use according to claim 1, wherein the amount of the metal-containing detergent of an alkali metal or alkaline earth metal salt of alkylphenol derivative having a Mannich base structure is in the range of 0.002 to 0.1 wt. % in terms of the nitrogen content, based on the total amount of the lubricating oil composition.

7. The use according to claim 1, wherein the amount of the phosphorus-containing organic compound is in the range of 0.01 to 0.2 wt. % in terms of the phosphorus content, based on the total amount of the lubricating oil composition.

8. The use according to claim 1, wherein the lubricating oil composition further comprises a metal-containing detergent selected from the group consisting of alkali metal or alkaline earth metal salicylates, carboxylates, phenates and sulfonates in an amount of 1.0 wt. % or less in terms of the metal content, based on the total amount of the lubricating oil composition.

9. The use according to claim 8, wherein the amount of the metal-containing detergent selected from the group consisting of alkali metal or alkaline earth metal salicylates, carboxylates, phenates and sulfonates and the amount of the metal-containing detergent of an alkali metal or alkaline earth metal salt of alkylphenol derivative having a Mannich base structure is in a ratio of 1:0.003 to 1:1 in terms of the metal content.

10. The use according to claim 1, wherein the lubricating oil composition further comprises a molybdenum compound selected from the group consisting of an oxymolybdenum complex prepared by the reaction between an acidic molybdenum compound and a basic nitrogen compound, sulfurized oxymolybdenum dithiocarbamate, and sulfurized oxymolybdenum dithiophosphate, in amount of 0.25 wt. % or less in terms of the molybdenum content, based on the total amount of the lubricating oil composition.

11. The use according to claim 1, wherein the lubricating oil composition further comprises an alkali metal borate in an amount of 2 wt. % or less, based on the total amount of the lubricating oil composition.

12. The use according to claim 1, wherein the lubricating oil composition further comprises an oxidation inhibitor selected from the group consisting of hindered phenol compounds and diarylamine compounds in an amount of 5 wt. % or less, based on the total amount of the lubricating oil composition.

13. The use according to claim 1, wherein the base oil contains 10 wt. % or more of a mineral oil showing the following characteristics:
- 17 wt. % or less evaporation loss according to ASTM D-5800,
- 90 wt. % or more saturated content,
- 10 wt. % or less, aromatic component,
- 0.01 wt. % or less, sulfur content, and
- 120 or more viscosity index.

14. The use according to claim 1, wherein the lubricating oil composition is a SAE viscosity grade selected from the group consisting of 0W20, 0W30, 5W20, 5W30 and 10W30.

15. The use according to claim 14, wherein the lubricating oil composition is a SAE viscosity grade of 10W30.

## Patentansprüche

1. Verwendung einer Schmierölzusammensetzung zum Verbessern der Kompatibilität mit Acrylgummidichtungen der Schmierölzusammensetzung im Betrieb eines Verbrennungsmotors, wobei die Schmierölzusammensetzung umfasst
a) eine größere Menge Basisöl mit Schmierviskosität,
b) ein stickstoffhaltiges aschefreies Dispergiermittel in einer Menge von 0,01 bis 0,3 Gew.-% im Sinne des Stickstoffgehalts, auf der Basis der Gesamtmenge der Schmierölzusammensetzung,
c) ein metallhaltiges Detergens eines Alkalimetall- oder Alkalierdmetallsalzes eines Alkylphenolderivats mit einer Mannichbasenstruktur in einer Menge von 0,001 bis 0,04 Gew.-% im Sinne des Metallgehalts, auf der Basis der Gesamtmenge der Schmierölzusammensetzung, und
d) eine phosphorhaltige organische Verbindung in einer Menge von 0,001 bis 0,5 Gew.-% im Sinne des Phosphorgehalts, auf der Basis der Gesamtmenge der Schmierölzusammensetzung,
wobei das Verhältnis der Bestandteile b) bis c) im Bereich von 1:0,005 bis 1:2 im Sinne des Stickstoffgehalts ist;
und wobei die Verbesserung der Kompatibilität mit Acrylgummidichtungen eine Verbesserung in Änderung der Verlängerung ist, gemessen mit Hilfe des CEC-L-39-T-96-Affinitätstests für Dichtungsgummi.

2. Verwendung gemäß Anspruch 1, wobei das stickstoffhaltige aschefreie Dispergiermittel ein Alkenyl- oder Alkylbernsteinsäureimid oder ein Derivat davon ist.

3. Verwendung gemäß Anspruch 1, wobei das metallhaltige Detergens eines Alkalimetall- oder Alkalierdmetallsalzes eines Alkylphenolderivats mit einer Mannichbasenstruktur durch die folgende Formel dargestellt wird: wobei R eine Alkylgruppe mit 8 bis 30 Kohlenstoffatomen ist und n 0 oder eine positive Ganzzahl.

4. Verwendung gemäß Anspruch 1, wobei die phosphorhaltige organische Verbindung ausgewählt ist aus der Gruppe Zinkdihydrocarbyldithiophosphate, Zinkdihydrocarbylphosphate, Phosphorsäureester, Phosphonsäureester und Thiophosphorsäureester.

5. Verwendung gemäß Anspruch 1, wobei die Menge stickstoffhaltiges aschefreies Dispergiermittel im Bereich von 0,01 bis 0,1 Gew.-% im Sinne des Stickstoffgehalts ist, auf der Basis der Gesamtmenge der Schmierölzusammensetzung.

6. Verwendung gemäß Anspruch 1, wobei die Menge metallhaltiges Detergens eines Alkalimetall- oder Alkalierdmetallsalzes eines Alkylphenolderivats mit einer Mannichbasenstruktur im Bereich von 0,002 bis 0,1 Gew.-% im Sinne des Stickstoffgehalts ist, auf der Basis der Gesamtmenge der Schmierölzusammensetzung.

7. Verwendung gemäß Anspruch 1, wobei die Menge phosphorhaltige organische Verbindung im Bereich von 0,01 bis 0,2 Gew.-% im Sinne des Phosphorgehalts ist, auf der Basis der Gesamtmenge der Schmierölzusammensetzung.

8. Verwendung gemäß Anspruch 1, wobei die Schmierölzusammensetzung zudem ein metallhaltiges Detergens umfasst, ausgewählt aus der Gruppe Alkalimetall- oder Alkalierdmetallsalicylate, -carboxylate, -phenate und -sulfonate in einer Menge von 1,0 Gew.-% oder weniger im Sinne des Metallgehalts, auf der Basis der Gesamtmenge der Schmierölzusammensetzung.

9. Verwendung gemäß Anspruch 8, wobei die Menge metallhaltiges Detergens, ausgewählt aus der Gruppe Alkalimetall- oder Alkalierdmetallsalicylate, -carboxylate, -phenate und -sulfonate und die Menge metallhaltiges Detergens eines Alkalimetall- oder Alkalierdmetallsalzes eines Alkylphenolderivats mit einer Mannichbasenstruktur in einem Verhältnis von 1:0,003 bis 1:1 im Sinne des Metallgehalts ist.

10. Verwendung gemäß Anspruch 1, wobei die Schmierölzusammensetzung zudem eine Molybdänverbindung umfasst, ausgewählt aus der Gruppe Oxymolybdänkomplex, hergestellt durch die Reaktion zwischen einer sauren Molybdänverbindung und einer basischen Stickstoffverbindung, sulfuriertes Oxymolybdändithiocarbamat und sulfuriertes Oxymolybdändithiophosphat, in einer Menge von 0,25 Gew.-% oder weniger im Sinne des Molybdängehalts, auf der Basis der Gesamtmenge der Schmierölzusammensetzung.

11. Verwendung gemäß Anspruch 1, wobei die Schmierölzusammensetzung zudem ein Alkalimetallborat in einer Menge von 2 Gew.-% oder weniger umfasst, auf der Basis der Gesamtmenge der Schmierölzusammensetzung.

12. Verwendung gemäß Anspruch 1, wobei die Schmierölzusammensetzung zudem einen Oxydationshemmer umfasst, ausgewählt aus der Gruppe gehinderte Phenolverbindungen und Diarylaminverbindungen in einer Menge von 5 Gew.-% oder weniger, auf der Basis der Gesamtmenge der Schmierölzusammensetzung.

13. Verwendung gemäß Anspruch 1, wobei das Basisöl 10 Gew.-% oder mehr eines Mineralös enthält mit den folgenden Eigenschaften:
- 17 Gew.-% oder weniger Verdunstungsverlust gemäß ASTM D-5800,
- 90 Gew.-% oder mehr gesättigter Gehalt,
- 10 Gew.-% oder weniger aromatischer Bestandteil,
- 0,01 Gew.-% oder weniger Schwefelgehalt, und
- Viskositätsindex von 120 oder mehr.

14. Verwendung gemäß Anspruch 1, wobei die Schmierölzusammensetzung einen SAE-Viskositätsgrad hat, ausgewählt aus der Gruppe 0W20, 0W30, 5W20, 5W30 und 10W30.

15. Verwendung gemäß Anspruch 14, wobei die Schmierölzusammensetzung einen SAE-Viskositätsgrad von 10W30 hat.

## Revendications

1. Utilisation d'une composition d'huile lubrifiante pour améliorer la compatibilité d'un joint en caoutchouc acrylique avec la composition d'huile lubrifiante pendant l'opération d'un moteur à combustion interne, où la composition d'huile lubrifiante comprend :
a) une quantité majeure d'une huile de base à viscosité lubrifiante,
b) un dispersant contenant de l'azote et sans teneur en cendres en une quantité de 0,01 à 0,3 pour cent en poids en termes du contenu en azote, sur la base du poids total de la composition d'huile lubrifiante,
c) un détergent contenant un métal d'un sel de métal alcalin ou alcalino-terreux d'un dérivé d'alkylphénole ayant une structure de base de Mannich en une quantité de 0,001 à 0,04 pour cent en poids en termes du contenu en métal, sur la base du poids total de la composition d'huile lubrifiante, et
d) un composé organique contenant du phosphore en une quantité de 0,001 à 0,5 pour cent en poids en termes du contenu en phosphore, sur la base du poids total de la composition d'huile lubrifiante,
où le rapport des composantes b) à c) est dans la plage entre 1:0,005 et 1:2 en termes du contenu en azote ;
et où l'amélioration de la compatibilité d'un joint en caoutchouc acrylique est une amélioration du change en élongation mesuré selon le test d'affinité CEC-L-39-T-96 pour les caoutchoucs d'étanchéité.

2. Utilisation selon la revendication 1, dans laquelle le dispersant contenant de l'azote et sans teneur en cendres est un imide succinique d'alcényle ou d'alkyle ou un de ses dérivés.

3. Utilisation selon la revendication 1, dans laquelle le détergent contenant un métal d'un sel de métal alcalin ou alcalino-terreux d'un dérivé d'alkylphénole ayant une structure de base de Mannich est représenté par la formule suivante : dans laquelle R est un groupe alkyle ayant 8 à 30 atomes de carbone, et n est 0 ou un nombre entier positif.

4. Utilisation selon la revendication 1, dans laquelle le composé organique contenant du phosphore est sélectionné parmi le groupe constitué par les dihydro-carbyldithiophosphates de zinc, les dihydrocarbylphosphates de zinc, les esters d'acide phosphorique, les esters d'acide phosphoreux, et les esters d'acide thiophosphorique.

5. Utilisation selon la revendication 1, dans laquelle la quantité du dispersant contenant de l'azote et sans teneur en cendres est dans la plage de 0,01 à 0,1 pour cent en poids en termes du contenu en azote, sur la base du poids total de la composition d'huile lubrifiante.

6. Utilisation selon la revendication 1, dans laquelle la quantité du détergent contenant un métal d'un sel de métal alcalin ou alcalino-terreux d'un dérivé d'alkylphénole ayant une structure de base de Mannich est dans la plage de 0,002 à 0,1 pour cent en poids en termes du contenu en azote, sur la base du poids total de la composition d'huile lubrifiante.

7. Utilisation selon la revendication 1, dans laquelle la quantité du composé organique contenant du phosphore est dans la plage de 0,01 à 0,2 pour cent en poids en termes du contenu en phosphore, sur la base du poids total de la composition d'huile lubrifiante.

8. Utilisation selon la revendication 1, dans laquelle la composition d'huile lubrifiante comprend en plus un détergent contenant un métal sélectionné parmi le groupe constitué par les salicylates, les carboxylates, les phénates et les sulfonates d'un métal alcalin ou métal alcalino-terreux en une quantité de 1,0 pour cent en poids ou moins en termes de contenu en métal, sur la base du poids total de la composition d'huile lubrifiante.

9. Utilisation selon la revendication 8, dans laquelle la quantité du détergent contenant un métal sélectionné parmi le groupe constitué par les salicylates, les carboxylates, les phénates et les sulfonates d'un métal alcalin ou métal alcalino-terreux et la quantité du détergent contenant un métal d'un sel de métal alcalin ou alcalino-terreux d'un dérivé d'alkylphénole ayant une structure de base de Mannich sont dans un rapport de 1:0,003 à 1:1 en termes du contenu en métal.

10. Utilisation selon la revendication 1, dans laquelle la composition d'huile lubrifiante comprend en plus un composé de molybdène sélectionné parmi le groupe constitué par un complexe oxymolybdène préparé par la réaction entre un composé de molybdène acide et un composé d'azote basique, un dithiocarbamate d'oxymolybdène sulfurisé, et un dithiophosphate d'oxymolybdène sulfurisé, en une quantité de 0,25 pour cent en poids ou moins en termes du contenu en molybdène, sur la base du poids total de la composition d'huile lubrifiante.

11. Utilisation selon la revendication 1, dans laquelle la composition d'huile lubrifiante comprend en plus un borate de métal alcalin en une quantité de 2 pour cent en poids ou moins, sur la base du poids total de la composition d'huile lubrifiante.

12. Utilisation selon la revendication 1, dans laquelle la composition d'huile lubrifiante comprend en plus un inhibiteur d'oxydation sélectionné parmi le groupe constitué par des composés stériquement empêchés et de diarylamine en une quantité de 5 pour cent en poids ou moins, sur la base du poids total de la composition d'huile lubrifiante.

13. Utilisation selon la revendication 1, dans laquelle l'huile de base comprend 10 pour cent en poids ou plus d'une huile minérale ayant les charactéristiques suivantes :
- 17 pour cent en poids ou moins de perte d'évaporation selon ASTM D-5800,
- 90 pour cent en poids ou plus de contenu saturé,
- 10 pour cent en poids ou moins de composante aromatique,
- 0,01 pour cent en poids ou moins de contenu en soufre, et
- un indice de viscosité de 120 ou plus.

14. Utilisation selon la revendication 1, dans laquelle la composition d'huile lubrifiante a un degré de viscosité SAE sélectionné parmi le groupe constitué par 0W20, 0W30, 5W20, 5W30 et 10W30.

15. Utilisation selon la revendication 14, dans laquelle la composition d'huile lubrifiante a un degré de viscosité SAE de 10W30.
